

## UNITED STATES PATENT OFFICE

2,056,810

## CELLULOUS MATERIAL

Frederic H. Smyser, Marblehead, Mass., assignor  
to General Electric Company, a corporation of  
New York

No Drawing. Application September 13, 1934,  
Serial No. 743,838

9 Claims. (Cl. 92—38)

The present invention relates to an improved process for treating cellulosic material and in particular waste cellulosic material such as bagasse and the like, in order to convert it into useful products and to the products produced thereby. More particularly the present invention is an improvement over the process described in my prior Patent No. 1,792,254 which is assigned to the assignee of the present invention.

10 In accordance with the process described in my prior patent above referred to comminuted cellulosic material such as waste bagasse, sawdust, cornstalks and the like is first treated under heat and pressure with an alkali such as sodium hydroxide whereby resinous substances formed from the natural constituents of the cellulosic material are caused to be intimately intermingled with the fibers thereof and then an acid such as sulfuric acid is added in order to precipitate the 15 resinous substances on and around the fibers. The mass, after filtering and washing is dried and then molded in a comminuted state in the presence of an alkaline agent.

I have discovered that I can eliminate the addition of the acid in order to precipitate the resinous substances on the fibers by controlling the original cooking of the cellulosic material. I have found that by carefully controlling the cooking of the material with the alkali solution using an 20 adjusted concentration of the latter a point is reached where the liquor turns sufficiently acid to precipitate the resinous substances on and around the fibers. This does away with the necessity of adding acid and eliminates the necessity of an 25 added handling operation. Moreover, the elimination of addition of acid yields a final product of superior dielectric strength since there is no excess acid to wash out which is always an expensive and uncertain operation. Since the acid 30 is not added to the mass as a separate entity the mass can be discharged directly into the filter for the washing operation which is now simpler, faster and less expensive.

In order that my invention may be better understood I cite an example below of my improved process. It is to be understood, however, that the example given is merely illustrative of my invention and is not limiting in character. The figures given in the example represent merely a 35 satisfactory balance between the amount of resin

formed, toughness of fiber and reasonable operating conditions as will readily be understood by those skilled in the art.

A charge consisting of

|                                 | Pounds | 5 |
|---------------------------------|--------|---|
| Bagasse fiber                   | 10     |   |
| Caustic soda (sodium hydroxide) | 1 1/8  |   |
| Water                           | 100    |   |

is placed in a digester which is sealed at atmospheric pressure. It is important that there be no leaks in the digester during the cooking operation as either an excess of air or a deficiency of air in the apparatus is detrimental. After sealing, the digester is heated to a temperature of 180 to 185° 10 C. for 18 to 22 hours. The temperature and time of cooking should be carefully observed since the effect of too long cooking or excess temperature will produce too much acid and result in a rotting of the fiber without formation of additional resin. 15 If the above temperature and time is observed it will be found that the liquor in the digester is acid to litmus and the mass is at the end point to be reached.

The mass is now allowed to cool and discharged 20 from the digester, placed in filters and the liquor allowed to drain off. The fiber is washed with water and dried. This fiber contains from 15 to 18% resin.

While it is not necessary to make the second 25 cook about to be described, it is preferred inasmuch as it enables the production of a fiber having a higher ultimate resin content.

The liquor drained from the fiber obtained from the digester is replaced therein and a fresh charge 30 of 10 lbs. of bagasse fiber is added, the digester is sealed and a second cook of from two to four hours is made at the same temperature as in the first case. At the end of this time, the material 35 in the digester is cooled and discharged therefrom, the liquor being drained and discarded. The fiber is thoroughly washed and dried. This fiber contains from 25 to 30% resin. While this lot of fiber may be used separately it is preferred to mix it with the first lot obtained in order to increase the average resin content of the mixed 40 fiber.

In my prior patent above referred to I molded the fiber in the presence of an alkaline agent. 45 In the present improvement I have found it ad- 50

vantageous to employ in place of the alkaline agent a heat convertible synthetic resin and preferably a water soluble phenolic resin prepared in the presence of an alkaline catalyst, for example, sodium carbonate ( $Na_2CO_3$ ) or hydroxide ( $NaOH$ ). By employing such a resin I am able to materially increase the water resistance, mechanical strength and dielectric properties of the finished product. Moreover, I do not need to employ a very large quantity of the resin in order to effect such improvements. Usually from 15 to 20% is sufficient.

The fiber so prepared may be molded under heat and pressure employing the usual ranges of 15 temperature and pressure employed in hot molding operations, allowance being made, of course, for the size, shape and any intricate design of the piece being molded. Fillers, dyes, pigments, strengthening agents, plasticizers and the like 20 may be added, if desired, before molding.

In some cases it may be desirable, for reasons of cost or other factors, to omit the addition of resin to the prepared fibers before molding. The material after treatment in the digester, and 25 washing and drying, may be comminuted or powdered and molded directly without the addition of any other substance whatever. Care must be exercised, however, in cooling the mold before the piece is removed therefrom.

30 If laminated material is desired, the prepared fiber, i. e., the fiber which has been taken from the digester and washed, is run into a beater, rod mill or other suitable apparatus where the fiber is prepared for a paper or board machine, and then 35 sheets formed according to standard paper or board making practice, after which the sheets are dried, laminated and molded. Any thickness of sheets may be molded employing the usual temperatures and pressures requisite for such operations. Since no thermosetting resins are 40 employed it is essential that the board be cooled in the press before withdrawal therefrom. If, however, the fiber having the water soluble phenolic resin added thereto is used a thermosetting 45 sheet may be made.

If desired a laminated product of the type described and claimed in Kienle and Scheiber Patent No. 1,921,757 may be made by following the procedure therein described for utilizing the fiber 50 produced in accordance with the present invention.

What I claim as new and desire to secure by Letters Patent in the United States:

1. A process for making a molded product from 55 cellulosic material containing natural substances capable of yielding resinous compounds therein, which comprises digesting said cellulosic material with an alkali solution of adjusted concentration at a temperature and for a time such that 60 the alkali is neutralized and until an acid reaction to litmus is obtained, and there is caused to precipitate on and around the fibers of the material certain resinous and resin forming constituents, separating the solid constituents, washing and 65 drying the same, adding a synthetic resin, and molding the mixture under heat and pressure.

2. A process for making a molded product which comprises preparing resinous compounds from waste cellulosic material containing natural 70 substances capable of yielding resinous compounds therein by treating the cellulosic material with alkali solution of adjusted concentration at a temperature and for a time sufficient to neutralize the alkali and to convert the liquor of 75 the mass from the alkaline to the acid side, wash-

ing, drying the mass so obtained, intimately mixing therewith a phenolic resin and molding under heat and pressure.

3. A process of making a molded product from 5 waste cellulosic material having natural substances capable of yielding resinous compounds therein which comprises treating such material solely with alkali solution of adjusted concentration under heat and pressure and at a temperature and for a time sufficient to neutralize the alkali to cause the resinous derivatives thereof to be intimately intermingled with the fibers thereof, adding a heat convertible resin, and molding under heat and pressure.

4. A process of making a molded product from 15 waste cellulosic material containing natural substances capable of yielding resinous compounds therein which comprises digesting said material with alkali solution of adjusted concentration under conditions of heat and pressure and at a 20 temperature and for a time sufficient to neutralize the alkali and to precipitate certain resinous substances formed therefrom on and around the fibers of the material, adding a phenolic resin to the mass before molding and molding under heat 25 and pressure.

5. A process for making a molded product which comprises the steps of digesting with caustic soda solution of adjusted concentration a 30 cellulosic material having natural substances capable of yielding resinous compounds therein until the dissolved resinous constituents are precipitated therefrom, filtering and washing the mass until it is neutral, drying the same, adding to the dried mass a water soluble phenolic resin, 35 reducing the entire mass to powdered form, and molding under heat and pressure.

6. The process of forming into a molded product a comminuted cellulosic material having natural substances capable of yielding resinous 40 compounds therein, which consists in digesting the cellulosic material with alkali solution of adjusted concentration to dissolve the binding substances and separate the cellulose fibers from each other, continuing the digesting operation 45 until the liquor has become acid and there has precipitated on and within the mass of fibers resinous and resin-forming substances, removing soluble by-products, adding a synthetic resin and molding under heat and pressure.

7. A process which comprises heating cellulosic material containing natural substances capable of yielding resinous substances therein, in a digester sealed at atmospheric pressure, with an alkali solution of adjusted concentration 55 for a time and at a temperature sufficient to neutralize the alkali and to convert the liquor to an acid reaction to litmus whereby the resinous substances formed from the natural substances of the cellulosic material are concentrated externally on and around the cellulosic fibers, cooling the mass, separating the fibers, washing and drying the latter, mixing a water soluble phenolic resin therewith, and heating under pressure in a closed die.

8. A process which comprises heating cellulosic material containing natural substances capable of yielding resinous compounds therein, in a digester sealed at atmospheric pressure with an alkali solution of adjusted concentration for 70 a time and at a temperature sufficient to neutralize the alkali and to convert the liquor to an acid reaction to litmus whereby the resinous substances formed from the natural substances of the cellulosic material are concentrated ex- 75

- ternally on and around the cellulosic fibers, cooling the mass, separating the fibers by removal of the liquor therefrom, digesting another batch of similar type cellulosic material with said liquor for a period considerably shorter than the first period of digestion, cooling the mass, separating the digested fibers, washing and drying the latter and combining it with the first batch of treated fibers, mixing a heat convertible phenolic resin therewith, and heating under pressure in a close die.
9. A process for making a laminated molded product which comprises digesting cellulosic ma-
- terial containing natural substances capable of yielding resinous compounds therein with an alkali solution until the alkali is neutralized and an acid reaction to litmus is obtained and there is caused to precipitate on and around the fibers of the material certain resinous and resin-forming constituents, separating the solid constituents, washing the same, forming a sheet therefrom in accordance with paper making practice, drying the sheet, and molding under heat and pressure the desired number of laminations of said sheet.

FREDERIC H. SMYSER.